# EUROPEAN PATENT SPECIFICATION

(11) **EP 2 518 175 B1**
(45) Date of publication and mention of the grant of the patent: **23.01.2019**
(21) Application number: 10839395.0
(22) Date of filing: 21.12.2010
(51) Int. Cl.: C22C 38/00, C21D 9/02, C22C 38/38, C22C 38/58, C21D 7/06

(54) **HIGH-STRENGTH SPRING STEEL**
HOCHFESTER FEDERSTAHL
ACIER À RESSORTS À HAUTE RÉSISTANCE

(30) Priority: 22.12.2009 JP 2009291143
(43) Date of publication of application: 31.10.2012
(73) Proprietor: Kabushiki Kaisha Kobe Seiko Sho, Chuo-ku Kobe-shi Hyogo 651-8585 (JP)
(72) Inventor: NAGAMATSU, Sayaka, Kobe-shi, Hyogo 657-0863 (JP); MARUO, Tomotada, Kobe-shi Hyogo 657-0863 (JP); YOSHIHARA, Nao, Kobe-shi Hyogo 657-0863 (JP)
(74) Representative: Müller-Boré & Partner Patentanwälte PartG mbB
(86) International application number: PCT/JP2010/073003
(87) International publication number: WO 2011/078165

(56) References cited:
- JP-A- 11 323 495
- JP-A- 2001 049 337
- JP-A- 2001 049 337
- JP-A- 2004 263 247
- JP-A- 2004 263 247
- JP-A- 2009 046 764
- SPIEKERMANN P: "LEGIERUNGEN - EIN BESONDERES PATENTRECHTLICHES PROBLEM? - LEGIERUNGSPRUEFUNG IM EUROPAEISCHEN PATENTAMT -", MITTEILUNGEN DER DEUTSCHEN PATENTANWAELTE, HEYMANN, KOLN, DE, 1 January 1993 (1993-01-01), pages 178-190, XP000961882, ISSN: 0026-6884
- PECKNER D ET AL: "HANDBOOK OF STAINLESS STEELS, PASSAGE", HANDBOOK OF STAINLESS STEELS, XX, XX, 1 January 1977 (1977-01-01), page 14.02, XP002053955,

## Description

The present invention relates to a spring steel useful as a raw material for a coil spring, and relates specifically to a spring steel used in manufacturing a coil spring and having the tensile strength of 1,900 MPa class under a condition as quenched.

With respect to a spring used for automobiles and the like (suspension spring and the like), weight reduction is required in order to reduce the exhaust gas and to improve the fuel consumption, and, as a part thereof, high-strengthening is directed to. In a high-strengthened spring, the sensitivity against a defect rises, breakage from a corrosion pit caused by adhesion of a snow melting agent is liable to occur for example, and early breakage due to corrosion fatigue becomes a problem. Therefore, a spring with high strength and excellent in corrosion fatigue property has been required. For example, "UHS1900" developed by the present applicant previously as a spring steel can achieve excellent corrosion fatigue property although the tensile strength is as high as 1,900 MPa class by performing quenching and tempering after coiling into a spring shape. Accordingly, a spring obtained from the spring steel can satisfy both the high strength and excellent corrosion fatigue property.

In general, such spring is manufactured by drawing of a spring steel (wire rod), cold-finishing, thereafter heating, hot-coiling, then quenching, tempering, and setting. The quenching and tempering treatment after hot-coiling is performed in order to adjust the strength of the spring. In the heat treatment such as the quenching and tempering treatment, much CO₂ is discharged. In recent years however, aiming to reduce the load against the earth environment, reduction of CO₂ has been strongly required as one of the global warming preventive measures. Therefore, even in the manufacturing steps for a coil spring, reduction of the discharge amount of CO₂ has been required.

Also, in the patent document 1, a steel for a stabilizer is proposed in which the toughness in the ordinary temperature and the toughness in the low temperature are improved by performing water-quenching soon after hot forming and being left as water-quenched without performing tempering. The steel for a stabilizer is featured that the componential composition is adjusted to a low C-high Mn-Cr system or a low C-high Mn-B-Cr system added with one element or two elements or more of Ti, V, Nb. The stabilizer which is the object of the patent document 1 is different in the technical field from that of a coil spring. For example, the strength level is 800 MPa class where the corrosion fatigue property does not become a problem, and the stabilizer is not related with the spring of a high strength range (1,900 MPa class for example) which is required to satisfy the corrosion fatigue property simultaneously.

Also, in general, the strength of iron and steel materials increases as the hardness increases, and, as the hardness increases, the toughness drops. That is, when the strength of the iron and steel materials increases, the toughness drops, however, as a material for a spring, a fracture property capable of enduring a severe use environment of a spring is required, and it becomes necessary to secure the toughness, or the low temperature toughness in particular which becomes important when used in a cold weather region, even in springs such as a high-strengthened suspension spring and the like.

For example, the patent document 2 discloses that the ductility and toughness were improved in a high-strength spring steel by adjusting various compositions, and the patent document 3 discloses that a spring steel having both of the hardness and toughness was obtained by adjusting various compositions. However, both of the patent documents 2 and 3 focused only on the toughness in the ordinary temperature, and did not consider the low temperature toughness. Usually, the toughness in the low temperature is inferior to the toughness in the ordinary temperature, and considering the ordinary temperature toughness disclosed in the patent documents 2 and 3, the low temperature toughness in the technology of the patent documents 2 and 3 is insufficient.

[Patent Document 1] Japanese Patent No. 4406341
[Patent Document 2] Japanese Patent No. 3577411
[Patent Document 3] Japanese Patent No. 3246733

Further, JP 2004-263247 A discloses a steel for a cold-formed spring which contains 0.36 to 0.46 mass% C. Also, JP 2001-049337 A discloses a method for producing a high-strength spring excellent in fatigue strength which contains 0.36 to 0.48 mass% C.

The present invention was developed considering such circumstances as described above, and its object is to provide a spring steel capable of manufacturing a coil spring achieving both of the high strength and excellent corrosion fatigue property as well as excellent in the low temperature toughness even when the tempering treatment after quenching is omitted in working into the coil spring. Also, another object of the present invention is to provide a spring obtained from the spring steel.

A high-strength spring steel in relation with the present invention that can solve the problems contains C: 0.15-0.33% (means mass%, hereinafter the same); Si: 1-3.5%; Mn: 0.20-2.0%; and contains at least one element selected from a group consisting of Ti: 0.005-0.10%, Nb: 0.005-0.05% and V: 0.05-0.25%; Cr: 0.05-1.20%; P: 0.030% or less; S: 0.02% or less; and optionally further containing Ni: 0.05-2% and Cu: 0.05-0.50%; and optionally further containing B: 0.005% or less and/or Mo: 0.60% or less with the remainder being iron and unavoidable impurities, in which a carbon equivalent Ceq₁ expressed by a formula (1) below is 0.55 or less. Ceq₁=[C]+0.108×[Si]·0.067×[Mn]+0.024×[Cr]-0.05×[Ni]+0.074×[V]...(1) (In the formula (1), each symbol in brackets represents the content (mass%) of the corresponding element.)

The spring steel of the present invention may contain Ni: 0.15-2%.

Further, it is also preferable that the spring steel of the present invention contains at least one element selected from a group consisting of Ti: 0.035-0.10%, Nb: 0.005-0.05%, and V: 0.05-0.25%, and the grain size number after quenching is 7.5 or above.

When the spring steel is used, the spring steel is hot-coiled, is quenched, and is thereafter subjected to setting while omitting tempering, a spring achieving both of the properties can be manufactured.

In the spring steel of the present invention, the element amount of a specific alloy element and the balance of mixing are properly controlled, therefore in manufacturing a coil spring using the spring steel, the tempering treatment after quenching can be omitted, and a spring achieving both of the high strength and excellent corrosion fatigue property and having excellent low temperature toughness in a state as quenched can be manufactured.

[FIG. 1] FIG. 1 is a graph showing the relation between the carbon equivalent (Ceq₁) and the time until the hydrogen embrittlement cracking of a specimen obtained in the example 1.
[FIG. 2] FIG. 2 is a graph showing the relation between the tensile strength and the low temperature toughness (vE-₅₀) of a specimen obtained in the example 2.

In manufacturing a spring by coiling a spring steel, the present inventors have repeatedly carried out intensive studies in order to provide a spring steel capable of manufacturing a spring achieving both of the high strength and excellent corrosion fatigue property as well as excellent in the low temperature toughness while omitting the tempering treatment after quenching performed after coiling. As a result, it was found out that, when the kind of the fundamental alloy elements contained in a spring steel was limited to C, Si, Mn, Cr, and at least an element out of Ti, Nb and V, or was limited to one in which the group of these elements was added further with (i) Ni and Cu or added further with (ii) B and/or Mo, and Si and Mn were positively contained while reducing the amount of C, Ti, Nb, V, Cr, Ni and Cu out of these elements as much as possible, the tempering treatment after quenching could be omitted in manufacturing a spring by coiling the spring steel, and a spring achieving both of the tensile strength of 1,900 MPa class and excellent corrosion fatigue property in a state as quenched as well as excellent in the low temperature toughness also achieved by more strictly adjusting the content of Ti, Nb and V could be provided, and the present invention was completed.

The spring steel of the present invention is characterized that the C amount in particular is reduced than the C amount used for an ordinary spring steel. By reducing the C amount, the amount of carbide precipitated in steel can be reduced, and therefore tempering after quenching which is performed in a usual spring manufacturing process can be omitted. That is, as described above, the spring is manufactured usually by drawing of a spring steel (wire rod), cold-finishing, thereafter heating, hot-coiling, then quenching, tempering, and setting. According to the necessity, shot peening is performed after setting, and painting is performed thereafter. However, because the C amount of the spring steel of the present invention is reduced, the strength of the spring can be secured even when setting is performed while omitting tempering after quenching.

On the other hand, in the spring steel of the present invention, Si and Mn are positively added. Si and Mn are easily obtainable elements, and stable supply is assured even when the amounts of Si and Mn are increased. Also, because Si and Mn have an action of enhancing the strength without dropping the toughness, both of the high strength and excellent corrosion fatigue property can be achieved by adding Si and Mn positively.

In order to surely achieve both of the high strength and excellent corrosion fatigue property based on the knowledge described above, it is necessary to strictly stipulate the amount of each element and to also stipulate the relation thereof. That is, in the present invention, the componential composition of the spring steel was designed as described below, and the carbon equivalent Ceq₁ expressed by the equation (1) below was made 0.55 or less. In the formula (1) below, each symbol in brackets represents the content (mass%) of the corresponding element.

### <Componential composition of spring steel>

The spring steel contains C: 0.15-0.33%, Si: 1-3.5%, Mn: 0.20-2.0%, and contains at least one element selected from a group consisting of Ti: 0.005-0.10%, Nb: 0.005-0.05% and V: 0.05-0.25%, and Cr: 0.05-1.20%. ${Ceq}_{1} = \left[C\right] + 0.108 \times \left[Si\right] - 0.067 \times \left[Mn\right] + 0.024 \times \left[Cr\right] - 0.05 \times \left[Ni\right] + 0.074 \times \left[V\right]$

The reason for setting the adding amount of each element and the reason for stipulating the carbon equivalent Ceq₁ are as described below.

The reason why C is made 0.15% or more is to enhance the quenchability and to secure the strength. Also, the reason why C is made 0.33% or less is to prevent deterioration of the toughness and corrosion fatigue property. The lower limit of the C amount is preferable to be 0.2% or more, more preferably 0.25% or more.

The reason why Si is made 1% or more is to make Si act as a solid solution strengthening element and to secure the strength. When Si is below 1%, the matrix strength is insufficient. On the other hand, when the Si amount becomes excessive, dissolution of carbide becomes insufficient in heating for quenching, heating at a higher temperature becomes necessary in order to make the steel austenitic uniformly, decarbonization of the surface progresses, and the fatigue property of the spring deteriorates. Therefore, by making Si 3.5% or less, decarbonization described above can be suppressed, occurrence of oxidation of the grain boundary and the like can be suppressed, and drop of the strength due to formation of an abnormal structure can be prevented. Si is preferable to be 1.5% or more and 3.0% or less, more preferably 1.80% or more and 2.5% or less.

By making Mn 0.20% or more, the quenchability can be enhanced and the strength can be secured. Also, by formation of sulfide-based inclusions, embrittlement of the grain boundary due to S can be prevented, and the toughness and corrosion fatigue property can be improved. Also, by making Mn 2.0% or less, a supercooled structure is generated, and deterioration of the toughness and corrosion fatigue property can be prevented. Furthermore, formation and coarsening of excessive sulfide-based inclusions can be suppressed, and deterioration of the toughness and corrosion fatigue property can be prevented. The lower limit of the Mn amount is preferable to be 0.5% or more, more preferably 0.80% or more, and the upper limit of the Mn amount is preferable to be 1.8% or less, and especially preferably 1.5% or less.

The reason why Ti is made 0.005% or more is to miniaturize the former austenite grains after quenching, to improve the strength and proof stress ratio, and to improve the toughness and corrosion fatigue property. By improving the toughness, the sag resistance can be improved. Also, the reason for making Ti 0.10% or less is to prevent precipitation of coarse inclusions (Ti-nitride for example) and to suppress deterioration of the corrosion fatigue property. The lower limit of the Ti amount is preferable to be 0.01% or more (especially preferable to be 0.05% or more), and the upper limit of the Ti amount is preferable to be 0.080% or less, more preferably 0.07% or less.

V is an element effectively acting for further enhancing the quenchability and enhancing the strength. Also, V is an element enhancing the toughness to contribute to improvement of the sag resistance, and miniaturizing the grains to improve the strength and proof stress ratio. In order to exert such actions, V is preferable to be contained by 0.05% or more, more preferably 0.08% or more, and further more preferably 0.1% or more. However, when V becomes excessive, coarse carbonitride is formed, and the toughness and corrosion fatigue property deteriorate. Accordingly, V is to be 0.25% or less, preferably 0.22% or less, and more preferably 0.2% or less.

Nb is an element enhancing the toughness to contribute to improvement of the sag resistance, and is an element miniaturizing the grains to improve the strength and proof stress ratio. In order to exert such actions, the Nb amount is to be made 0.005% or more, preferably 0.008% or more, and more preferably 0.01% or more. On the other hand, when the Nb amount becomes excessive, the toughness is influenced adversely. Accordingly, the Nb amount is to be 0.05% or less, preferably 0.04% or less, and more preferably 0.03% or less.

Ti, V and Nb may be added solely, or may be added combining two elements or more. The content of Ti, V and Nb is preferable to be Ti: 0.035-0.10%, Nb: 0.005-0.05%, V: 0.05-0.25% respectively, and it is to contain at least one element thereof. Also, by containing Ti, V and Nb by these ranges, the grain miniaturizing effect can be effectively exerted, and the grain size number after quenching can be made 7.5 or above, which results in exertion of excellent low temperature toughness. The grain size number after quenching is preferable to be 8.0 or above, more preferably 9.0 or above. The low temperature toughness of the spring steel of the present invention is, for example, 50J/cm² or more in terms of Charpy absorbed energy at -50°C, preferably 70 J/cm² or more, and more preferably 80 J/cm² or more.

By making Cr 0.05% or more, the steel matrix is strengthened by strengthening solid solution, the quenchability is improved, and the strength can be secured. Also, Cr is an element making the rust formed on the surface layer part under a corroding condition amorphous and dense and contributing to improvement of the corrosion resistance. On the other hand, by making Cr 1.20% or less, drop of the Ms point and formation of a supercooled structure are prevented, the toughness and corrosion fatigue property can be secured, and reduction of the strength and hardness due to insufficient dissolution of Cr-carbide in quenching can be prevented. Cr is preferable to be 0.1% or more and 1.10% or less, more preferably 0.5% or more and 1.05% or less.

The remainder of the spring steel of the present invention is substantially iron. However, it is rightly allowed that the unavoidable impurities brought in due to the situation of the material such as the iron material (including scraps), auxiliary raw material, and the like as well as the manufacturing facilities and the like are included in the steel. Out of the unavoidable impurities, it was stipulated particularly that P was to be 0.030% or less and S was to be 0.02% or less. The reason why such ranges were stipulated is as described below.

The reason why P is made 0.030% or less is to suppress segregating on the former austenite grain boundary and making the grain boundary brittle and to prevent deterioration of the toughness and corrosion fatigue property. P is preferable to be 0.02% or less, more preferably 0.01% or less. Although P is preferable to be as little as possible, it is usually included by approximately 0.001%.

The reason why S is made 0.02% or less is to prevent that sulfide-based inclusions are formed in the steel, coarsened, and deteriorate the corrosion fatigue property. S is preferable to be 0.015% or less, especially preferably 0.01% or less. Similar to P, S is also preferable to be as little as possible, however it is usually included by approximately 0.001%.

The total amount of P and S is preferable to be 0.015% or less, more preferably 0.010% or less.

The reason why the carbon equivalent Ceq₁ is made 0.55 or less is to achieve both of the strength and corrosion fatigue property of the spring even when the tempering treatment after quenching is omitted in manufacturing a coil spring by coiling the spring steel. That is, the carbon equivalent Ceq₁ represents the contribution degree of an alloy element exerting influence on the hardness after quenching, the hardness of the core part of the spring can be secured by omitting the tempering treatment after quenching while reducing the value, and high strengthening can be achieved. Also, by suppressing the carbon equivalent Ceq₁ to 0.55 or less, the degree of dependability of the alloy element can be lowered, and stable supply can be ensured more. The carbon equivalent Ceq₁ is preferable to be 0.53 or less, more preferably 0.50 or less. Also, the cost can be reduced as the composition is designed so that the carbon equivalent Ceq₁ becomes as small as possible, however, in order to achieve both of the strength and corrosion fatigue property, it is necessary to add alloy elements to some degree. Therefore, the lower limit of the carbon equivalent Ceq₁ is 0.30. Also, in calculation of the formula (1) below, when there is an element not contained, calculation should be executed assuming that the content of the element is 0 mass%.

The spring steel of the present invention is to satisfy the chemical componential composition and the carbon equivalent Ceq₁, however aiming to further improve the property, Ni and Cu may be contained, and B and/or Mo may also be contained.

When Ni and Cu are to be contained (that is, using both of Ni and Cu simultaneously), the Ni amount is to be 0.05-2%, and the Cu amount is to be 0.05-0.50%. The reason why Ni is made 0.05% or more is to enhance the toughness, to lower the defect sensitivity, and to improve the corrosion fatigue property. Also, Ni has an action of making the rust formed amorphous and dense to improve the corrosion resistance, and has also an action of improving the setting resistance which is important as the spring property. On the other hand, by making Ni 2% or less, dropping of the Ms point and formation of a supercooled structure can be prevented, and the toughness and corrosion fatigue property can be secured. Ni is preferable to be 0.15% or more and 2% or less, more preferably 0.18% or more and 1.5% or less, further more preferably 0.20% or more and 1% or less, especially 0.5% or less.

Because Cu is an element electrochemically nobler than iron, it is an element having an action of making the rust dense and improving the corrosion resistance. Therefore, when Cu is contained, the Cu amount is to be 0.05% or more. However, even if Cu is added excessively, its effect saturates, and embrittlement of the raw material due to hot rolling may be caused adversely. Accordingly, the upper limit of the Cu amount was made 0.50% or less. Cu is preferable to be 0.1% or more and 0.4% or less, more preferably 0.15% or more (especially 0.18% or more) and 0.3% or less.

B is an element enhancing the quenchability further to enhance the grain boundary strength, enhancing the toughness to improve the setting resistance, and making the rust formed on the surface dense to improve the corrosion resistance. In order to exert such actions, B is preferable to be contained by 0.0005% or more, more preferably 0.001% or more, and further more preferably 0.0015% or more. However, when B becomes excessive, the effects saturate and coarse carbonitride is formed, and the toughness and corrosion fatigue property deteriorate. Therefore, B is to be 0.005% or less, preferably 0.004% or less, and more preferably 0.003% or less.

Mo is an element enhancing the toughness and contributing to improvement of the setting resistance, and is an element securing the quenchability and enhancing the strength and toughness of the steel. In order to exert such actions effectively, the Mo amount is preferable to be 0.05% or more, more preferably 0.08% or more, and further more preferably 0.10% or more. On the other hand, even if the Mo amount becomes excessive, the effects saturate. Therefore, the Mo amount is to be 0.60% or less, more preferably 0.50% or less, and further more preferably 0.35% or less. B and Mo may be contained solely, or both may be used simultaneously.

As described above, the spring steel of the present invention is characterized that the amount of each alloy element is strictly stipulated and the relation thereof is stipulated, and when the spring steel is used, the tempering treatment after quenching performed after coiling can be omitted, and the spring achieving both of the high strength of 1,900 MPa or above tensile strength even in a state as quenched and excellent corrosion fatigue property can be manufactured. Also, by more strictly controlling the content of the elements having a grain miniaturizing action (Ti, Nb and V), the low temperature toughness can be improved. Below, a method for manufacturing a spring from the spring steel will be described.

In manufacturing a spring from the spring steel of the present invention, it is necessary to omit tempering after quenching. That is, although the process is the same with that of the prior art including the steps of drawing of a spring steel (wire rod) satisfying the chemical componential composition, cold-finishing, thereafter heating, hot-coiling to form into a spring shape, and quenching, it is necessary to perform setting while omitting tempering after quenching. Because the C amount of the spring steel of the present invention is reduced than that of the spring steel of the prior arts, when tempered after quenching, the spring steel is softened excessively, and the toughness and corrosion fatigue property deteriorate. Accordingly, it is necessary to omit tempering after quenching.

Here, "omission of tempering" means the spring is not heated to a temperature exceeding 350°C after quenching.

The setting may be performed either in a cold state or in a warm state. The temperature of cold setting can be an ordinary temperature, and the temperature of warm setting can be approximately 200-250°C.

After setting, painting may be performed after shot peening according to the necessity. The condition of shot peening and painting is not limited particularly, and the ordinary condition can be employed.

The spring thus obtained can achieve both of the high strength and excellent corrosion fatigue property, and is excellent in the low temperature toughness as well.

The manufacturing condition of the spring steel in relation with the present invention is not particularly limited, however in order to make the grain size number 7.5 or above which is a preferable aspect of the present invention, it is recommendable to make the heating temperature before quenching 925°C or below and to make the heating time 15 min or less. The lower limits of the heating temperature before quenching and the heating time are not particularly limited, however the lower limit of the heating temperature is approximately 850°C, and the lower limit of the heating time is approximately 10 min usually.

### [Examples]

Although the present invention will be described below more specifically referring to examples, the present invention is not to be limited by the examples described below, it is a matter of course that the present invention can also be implemented with modifications added appropriately within the range adaptable to the purposes described previously and later, and any of them is to be included within the technical range of the present invention.

### Example 1

After the steel of the chemical componential composition shown in Table 1 below (the remainder is iron and unavoidable impurities) was molten by a vacuum melting furnace of 150 kg, the steel was held at 1,200°C, was thereafter hot forged into a billet of 155 mm square, the billet was hot-rolled, and the spring steel with 13.5 mm diameter (wire rod for a spring) was manufactured. The wire rod for a spring was subjected to finish-rolling so that the diameter became 12.5 mm, was thereafter cut to the length of 70 mm, and was then quenched. Quenching was performed by heating for 10 min at the temperature of 925°C, and thereafter being dipped into an oil bath with the temperature of 50°C. After quenching, a specimen of 10 mm width×1.5 mm thickness×65 mm length was cut out by machining.

No. 29 and No. 30 shown in Table 1 are the data imitating the wire rod for a spring "UHS1900" made by Kobe Steel, Ltd., and in No. 30 out of them, the specimen was manufactured by quenching, thereafter tempering by being held for 1 hour at 400°C, and then being machined in a condition the same with the above. Table 2 shows whether tempering was performed or not.

Also, the chemical componential amount in the steel and the calculation result of the carbon equivalent (Ceq₁) calculated from the formula (1) are shown in Table 1 below.

The strength and corrosion fatigue property of the specimen obtained were examined as described below.

The strength and corrosion fatigue property of the specimen were measured imitating that setting was performed in a cold state or in a warm state. That is, when cold setting was imitated, the specimen was used for each test as it was, and when warm setting was imitated, the specimen heated for 60 min at 200°C was used for each test. Table 2 below shows which of cold setting and warm setting was imitated.

### <Strength>

The strength of the specimen was evaluated by measuring the hardness of the specimen with a Rockwell hardness tester using the C scale. The measurement result of the C hardness is shown in Table 2 below. In the present invention, those with HRC of 51 or more are to be evaluated to have passed.

### <Corrosion fatigue property>

The corrosion fatigue property was evaluated by performing a hydrogen embrittlement cracking test. In the hydrogen embrittlement cracking test, the specimen was immersed in the aqueous solution of a mixture of sulfuric acid (0.5 mol/L) and potassium thiocyanate (KSCN: 0.01 mol/L) while applying the stress of 1,400 MPa on the specimen by 4-point bending, the voltage of -700 mV which is lower than the SCE electrode was applied using a potentiostat, and the time until cracking occurred (hereinafter referred to as "the time until hydrogen embrittlement cracking") was measured. The measurement result of the hydrogen embrittlement cracking test is shown in Table 2 below. In the present invention, those in which the time until cracking occurs is 600 sec or more are evaluated to have passed.

Also, the criteria of 51 or above of HRC and 600 sec or more of the time until cracking occurs mean to have the property equal or better than that of a suspension spring according to the prior art (No. 30 of the Table 2 below) obtained performing tempering after quenching.

In FIG. 1, the relation between the carbon equivalent (Ceq₁) and the time until hydrogen embrittlement cracking (sec) is shown. In FIG. 1, the results of No. 1-15, 31, 33 were shown by □, the results of No. 16-29, 32 were shown by **●,** and the result of No. 30 (with tempering) was shown by ∘.

As is clear from FIG. 1, it is known that there is a tendency that, as the carbon equivalent (Ceq₁) is reduced, the time until hydrogen embrittlement cracking can be made longer and the corrosion fatigue property can be improved.

From Table 2, the following study is possible.

No. 30 is an example in which tempering was performed after quenching. In the example, the hardness of the core part was secured, the strength was high, the time until hydrogen embrittlement cracking was excellent, and the corrosion fatigue property was improved. However, because the tempering treatment was performed after quenching, the discharge amount of CO₂ could not be reduced.

Although the componential composition of No. 29 is similar to that of the No. 30, it is an example of omitting tempering after quenching. In the example, because the tempering treatment is omitted, the discharge amount of CO₂ can be reduced, however, because the carbon equivalent exceeds 0.55 and tempering is omitted in spite that the amount of the alloy element is much, the hardness of the core part becomes too hard, the toughness drops, the time until hydrogen embrittlement cracking becomes short, and the corrosion fatigue property deteriorates.

No. 16-28, 32 are the examples not satisfying the requirement stipulated in the present invention, and the high strength and excellent corrosion fatigue property were not achieved simultaneously. That is, the carbon equivalent (Ceq₁) of the spring steel exceeded the range stipulated in the present invention, tempering after quenching was omitted, and the discharge amount of CO₂ therefore could be reduced, however the hardness of the core part became too hard, the toughness dropped, the time until hydrogen embrittlement cracking became short, and the corrosion fatigue property deteriorated.

No. 1, 4, 13 and 15 are reference examples not satisfying the requirement stipulated in the present invention. No. 2, 3, 5-12, 14 and 33 are the examples satisfying the requirement stipulated in the present invention, and both of the high strength and excellent corrosion fatigue property were achieved. That is, while the carbon equivalent (Ceq₁) was suppressed to 0.55 or below, the discharge amount of CO₂ could be reduced because tempering after quenching was omitted, the hardness of the core part could be secured appropriately, and the high strength was achieved. Also, the time until hydrogen embrittlement cracking was long, and the corrosion fatigue property was also improved. Furthermore, because the carbon equivalent (Ceq₁) of the spring steel was suppressed to 0.55 or below, the degree of dependability of the alloy element can be lowered, and stable supply can be achieved. Accordingly, it is known that, when the spring steel of the present invention is used, a spring exerting the property of the same level with the No. 30 imitating the "UHS1900" or higher can be provided.

**[Table 1]**

| No. | Chemical corrposition (mass%) | | | | | | | | | | | | | Carbon equivalent (mass%) |
|---|---|---|---|---|---|---|---|---|---|---|---|---|---|---|
| | C | Si | Mn | Ni | Cr | Ti | Cu | P | S | V | B | P+S | Others | |
| 1 | 0.34 | 1.90 | 0.25 | 0.58 | 1.00 | 0.081 | 0.23 | 0.003 | 0.008 | - | - | 0.011 | | 0.52 |
| 2 | 0.33 | 1.76 | 0.21 | 0.40 | 1.07 | 0.061 | 0.28 | 0.002 | 0.004 | - | - | 0.006 | | 0.51 |
| 3 | 0.33 | 1.76 | 0.21 | 0.37 | 1.08 | 0.060 | 0.28 | 0.001 | 0.004 | 0.160 | - | 0.005 | | 0.53 |
| 4 | 0.34 | 1.77 | 0.21 | 0.33 | 1.06 | 0.060 | 0.28 | 0.001 | 0.005 | 0.158 | - | 0.006 | | 0.54 |
| 5 | 0.33 | 2.01 | 1.21 | 0.20 | 0.05 | 0.031 | 0.20 | 0.003 | 0.005 | - | 0.002 | 0.008 | | 0.46 |
| 6 | 0.15 | 2.20 | 1.00 | 0.25 | 0.20 | 0.090 | 0.25 | 0.015 | 0.005 | - | - | 0.020 | | 0.31 |
| 7 | 0.29 | 3.00 | 1.70 | 0.20 | 0.05 | 0.032 | 0.20 | 0.003 | 0.005 | - | - | 0.008 | | 0.49 |
| 8 | 0.29 | 2.17 | 0.78 | 0.20 | 0.20 | 0.073 | 0.16 | 0.007 | 0.004 | - | - | 0.011 | | 0.47 |
| 9 | 0.29 | 1.76 | 0.21 | 0.30 | 1.06 | 0.061 | 0.28 | 0.001 | 0.003 | 0.161 | - | 0.004 | | 0.49 |
| 10 | 0.15 | 2.20 | 1.00 | 0.25 | 0.20 | 0.090 | 0.25 | 0.015 | 0.005 | - | 0.002 | 0.020 | | 0.31 |
| 11 | 0.28 | 2.01 | 0.48 | 0.26 | 1.05 | 0.060 | 0.21 | 0.002 | 0.006 | 0.158 | 0.002 | 0.008 | | 0.49 |
| 12 | 0.16 | 2.01 | 0.80 | 0.25 | 1.06 | 0.061 | 0.21 | 0.009 | 0.007 | 0.157 | 0.002 | 0.016 | | 0.35 |
| 13 | 0.40 | 2.01 | 1.20 | 0.19 | 0.05 | 0.031 | 0.20 | 0.006 | 0.005 | - | 0.002 | 0.011 | | 0.53 |
| 14 | 0.29 | 2.01 | 1.21 | 0.20 | 0.05 | 0.031 | 0.20 | 0.007 | 0.006 | - | 0.002 | 0.013 | | 0.42 |
| 15 | 0.40 | 2.01 | 1.20 | 0.19 | 0.05 | 0.031 | 0.20 | 0.006 | 0.005 | - | 0.002 | 0.011 | | 0.53 |
| 16 | 0.60 | 1.73 | 0.88 | 0.08 | 0.20 | - | 0.19 | 0.010 | 0.019 | 0.154 | - | 0.029 | Nb.0.020. Mo:0.03 | 0.74 |
| 17 | 0.48 | 1.82 | 0.21 | 0.15 | 1.48 | 0.072 | 0.20 | 0.006 | 0.006 | 0.204 | - | 0.012 | | 0.71 |
| 18 | 0.54 | 1.81 | 0.20 | 0.34 | 1.25 | 0.077 | 0.42 | 0.006 | 0.008 | 0.098 | - | 0.014 | | 0.74 |
| 19 | 0.45 | 1.86 | 0.15 | 0.50 | 0.96 | 0.050 | 0.19 | 0.003 | 0.003 | 0.104 | - | 0.006 | | 0.65 |
| 20 | 0.48 | 2.08 | - | 0.78 | 1.50 | 0.091 | 0.69 | 0.007 | 0.002 | - | - | 0.009 | Nb:0.002 | 0.70 |
| 21 | 0.49 | 2.10 | 0.18 | 0.67 | 1.22 | 0.093 | 0.52 | 0.004 | 0.004 | - | - | 0.008 | | 0.70 |
| 22 | 0.48 | 2.10 | 0.32 | 0.73 | 1.12 | 0.072 | 0.20 | 0.007 | 0.005 | - | - | 0.012 | | 0.68 |
| 23 | 0.48 | 2.08 | 0.36 | 0.70 | 1.06 | 0.075 | 0.19 | 0.003 | 0.004 | 0.100 | - | 0.007 | | 0.68 |
| 24 | 0.42 | 1.92 | 0.15 | 0.58 | 1.02 | 0.080 | 0.23 | 0.025 | 0.002 | 0.184 | - | 0.027 | | 0.63 |
| 25 | 0.40 | 2.27 | 1.01 | 0.25 | 0.21 | 0.089 | 0.26 | 0.032 | 0.005 | - | - | 0.037 | | 0.57 |
| 26 | 0.42 | 2.24 | 1.01 | 0.25 | 0.21 | 0.088 | 0.26 | 0.040 | 0.004 | - | 0.002 | 0.044 | | 0.59 |
| 27 | 0.41 | 2.17 | 0.79 | 0.25 | 0.21 | 0.010 | 0.27 | 0.014 | 0.004 | - | 0.002 | 0.018 | | 0.58 |
| 28 | 0.42 | 2.27 | 1.21 | 0.25 | 0.20 | 0.015 | 0.26 | 0.012 | 0.005 | - | - | 0.017 | | 0.58 |
| 29 30 | 0.41 | 1.79 | 0.16 | 0.44 | 1.06 | 0.063 | 0.26 | 0.007 | 0.003 | 0.154 | - | 0.010 | | 0.61 |
| | 0.41 | 1.75 | 0.18 | 0.51 | 1.05 | 0.070 | 0.21 | 0.009 | 0.004 | 0.160 | - | 0.013 | | 0.61 |
| 31 | 0.38 | 1.71 | 0.85 | 0.06 | 1.02 | 0.052 | 0.21 | 0.003 | 0.006 | 0.104 | | 0.009 | | 0.54 |
| 32 | 0.39 | 2.98 | 1.70 | 0.21 | 0.05 | 0.035 | 0.21 | 0.007 | 0.005 | | 0.002 | 0.012 | | 0.59 |
| 33 | 0.32 | 2.06 | 1.22 | | 0.05 | 0.038 | | 0.008 | 0.006 | | | 0.014 | | 0.46 |

**[Table 2]**

| No. | With/without tempering | Setting | Hardness (HRC) | Time until hydrogen embrittlement cracking (sec) |
|---|---|---|---|---|
| 1 | Without | Cold | 55.9 | 717 |
| 2 | Without | Cold | 55.8 | 613 |
| 3 | Without | Cold | 55.6 | 844 |
| 4 | Without | Cold | 56.0 | 797 |
| 5 | Without | Cold | 55.3 | 876 |
| 6 | Without | Cold | 51.4 | 1800 |
| 7 | Without | Cold | 54.6 | 1797 |
| 8 | Without | Cold | 55.5 | 1280 |
| 9 | Without | Cold | 55.3 | 1188 |
| 10 | Without | Cold | 51.1 | 1800 |
| 11 | Without | Cold | 55.2 | 1235 |
| 12 | Without | Cold | 51.3 | 1800 |
| 13 | Without | Cold | 56.2 | 1562 |
| 14 | Without | Warm | 54.2 | 1640 |
| 15 | Without | Warm | 56.1 | 1510 |
| 16 | Without | Cold | 61.3 | 40 |
| 17 | Without | Cold | 59.5 | 38 |
| 18 | Without | Cold | 61.3 | 48 |
| 19 | Without | Cold | 58.5 | 466 |
| 20 | Without | Cold | 58.7 | 114 |
| 21 | Without | Cold | 59.0 | 164 |
| 22 | Without | Cold | 58.7 | 144 |
| 23 | Without | Cold | 59.7 | 246 |
| 24 | Without | Cold | 56.0 | 226 |
| 25 | Without | Cold | 55.7 | 355 |
| 26 | Without | Cold | 55.5 | 128 |
| 27 | Without | Cold | 55.9 | 284 |
| 28 | Without | Cold | 56.0 | 411 |
| 29 | Without | Cold | 55.8 | 575 |
| 30 | With | Cold | 52.2 | 603 |
| 31 | Without | Cold | 55.5 | 954 |
| 32 | Without | Cold | 56.8 | 579 |
| 33 | Without | Cold | 55.2 | 925 |

### Example 2

After the steel of the chemical componential composition shown in Table 3 (the remainder is iron and unavoidable impurities) was molten by a vacuum melting furnace of 150 kg, the steel was casted by an ingot-making method or a continuous casting method, a billet of 155 mm square was manufactured thereafter by a blooming mill, was hot-rolled into a wire rod with the diameter of 13.5 mm which was made a test material. These test materials were heated for 10 min at the temperature of 925°C, and were thereafter put into an oil bath of 50°C for quenching. Only No. 2-24 was subjected to tempering treatment for 1 hour at 400°C after quenching.

**[Table 3]**

| **No.** | Chemical composition (mass%) | | | | | | | | | | | | Carbon equivalent (mass% ) |
|---|---|---|---|---|---|---|---|---|---|---|---|---|---|
| | **C** | **Si** | **Mn** | **Cr** | **V** | **Ti** | **P** | **S** | **Ni** | **Cu** | **P+S** | Others | |
| **2-1** | **0.30** | **3.00** | **1.70** | **0.05** | | **0.037** | **0.003** | **0.005** | **0.20** | **0.20** | **0.008** | | **0.50** |
| **2-2** | **0.30** | **2.01** | **1.21** | **0.05** | | **0.036** | **0.003** | **0.005** | **0.20** | **0.20** | **0.008** | **B:0.002** | **0.43** |
| **2-3** | **0.15** | **2.20** | **1.00** | **0.20** | **0.180** | **0.090** | **0.010** | **0.005** | **0.25** | **0.25** | **0.015** | | **0.33** |
| **2-4** | **0.15** | **2.20** | **1.00** | **0.20** | | **0.090** | **0.010** | **0.005** | **0.25** | **0.25** | **0.015** | **B:0.002** | **0.31** |
| **2-5** | **0.34** | **2.15** | **1.00** | **0.38** | | **0.098** | **0.009** | **0.006** | **0.24** | **0.22** | **0.015** | **Nb:0.01** | **0.50** |
| **2-6** | **0.34** | **2.21** | **1.15** | **0.65** | **0.150** | **0.072** | **0.005** | **0.005** | **0.20** | **0.31** | **0.010** | **Mo:0.23** | **0.52** |
| **2-7** | **0.38** | **1.76** | **0.86** | **1.08** | **0.160** | **0.060** | **0.001** | **0.004** | **0.37** | **0.28** | **0.005** | | **0.53** |
| **2-8** | **0.34** | **1.76** | **0.86** | **1.06** | **0.161** | **0.061** | **0.001** | **0.003** | **0.30** | **0.28** | **0.004** | **B:0.001** | **0.49** |
| **2-9** | **0.37** | **1.79** | **0.82** | **1.06** | **0.170** | **0.068** | **0.002** | **0.006** | **0.53** | **0.22** | **0.008** | | **0.52** |
| **2-10** | **0.37** | **1.87** | **0.80** | **0.98** | **0.107** | **0.052** | **0.002** | **0.004** | **0.51** | **0.06** | **0.006** | | **0.52** |
| **2-11** | **0.38** | **1.75** | **0.84** | **1.05** | **0.160** | **0.074** | **0.006** | **0.003** | **0.51** | **0.48** | **0.009** | | **0.52** |
| **2-12** | **0.34** | **1.79** | **0.81** | **1.06** | **0.154** | **0.063** | **0.005** | **0.003** | **0.44** | **0.06** | **0.008** | | **0.49** |
| **2-13** | **0.35** | **1.75** | **0.82** | **1.09** | | **0.041** | **0.004** | **0.004** | **0.77** | **0.21** | **0.008** | | **0.47** |
| **2-14** | **0.38** | **1.71** | **0.85** | **1.02** | **0.104** | **0.052** | **0.003** | **0.006** | **0.06** | **0.21** | **0.009** | | **0.54** |
| **2-15** | **0.60** | **1.73** | **0.88** | **0.20** | **0.154** | | **0.010** | **0.019** | **0.08** | **0.19** | **0.029** | **Mo:0.13, Nb:0.02** | **0.74** |
| **2-16** | **0.52** | **1.89** | **0.15** | **1.01** | **0.179** | **0.078** | **0.003** | **0.023** | **0.29** | **0.23** | **0.026** | | **0.74** |
| **2-17** | **0.46** | **2.18** | **0.79** | **0.21** | | **0.071** | **0.005** | **0.004** | | | **0.009** | | **0.65** |
| **2-18** | **0.46** | **2.20** | **0.41** | **0.21** | | **0.072** | **0.007** | **0.004** | **0.30** | | **0.011** | | **0.66** |
| **2-19** | **0.45** | **2.18** | **0.77** | | | **0.069** | **0.005** | **0.005** | **0.20** | **0.31** | **0.010** | | **0.62** |
| **2-20** | **0.40** | **2.21** | **0.82** | **0.15** | | | **0.005** | **0.005** | **0.20** | **0.31** | **0.010** | | **0.58** |
| **2-21** | **0.30** | **3.00** | **1.70** | **0.05** | | | **0.010** | **0.005** | **0.20** | **0.20** | **0.015** | | **0.50** |
| **2-22** | **0.30** | **2.01** | **1.21** | **0.05** | | | **0.012** | **0.005** | **0.20** | **0.20** | **0.017** | **B:0.002** | **0.43** |
| **2-23** | **0.54** | **1.50** | **0.70** | **0.70** | | | **0.012** | **0.006** | | | **0.018** | | **0.67** |
| **2-24** | **0.54** | **1.50** | **0.70** | **0.70** | | | **0.012** | **0.006** | | | **0.018** | | **0.67** |
| **2-25** | **0.32** | **2.06** | **1.22** | **0.05** | | **0.038** | **0.008** | **0.006** | | | **0.014** | | **0.46** |
| **2-26** | **0.39** | **2.98** | **1.70** | **0.05** | | **0.035** | **0.007** | **0.005** | **0.21** | **0.21** | **0.012** | **B:0.002** | **0.59** |

### <Low temperature toughness>

An impact test specimen with 2 mm U-notch was taken from the test material after the quenching, and the Charpy absorbed energy at -50°C (vE₋₅₀) was obtained according to JIS Z 2242. The tests were carried out on two pieces for each steel kind, and the average value thereof was made the Charpy absorbed energy of each steel kind.

### <Grain size number>

At the D/4 position (D is the diameter of the wire rod) of the test material after the quenching, an optional area of 15 mm² was observed with an optical microscope (magnification: 400 times), and the grain size number was measured according to JIS G 0551. The measurement was performed on two fields of view, and the average value thereof was made the austenite grain size.

The result is shown in Table 4.

**[Table 4]**

| **No.** | Grain size number | Charpy absorbed energy **vE₋₅₀(J/cm²)** | Tensile strength **TS (MPa)** |
|---|---|---|---|
| **2-1** | **7.5** | **67.7** | **1726** |
| **2-2** | **8.5** | **65.7** | **1534** |
| **2-3** | **8.7** | **91.8** | **1109** |
| **2-4** | **7.8** | **68.0** | **1137** |
| **2-5** | **9.0** | **60.9** | **1833** |
| **2-6** | **8.2** | **68.4** | **1710** |
| **2-7** | **9.5** | **81.3** | **1804** |
| **2-8** | **10.0** | **85.7** | **1638** |
| **2-9** | **10.8** | **85.8** | **1897** |
| **2-10** | **9.5** | **86.5** | **1982** |
| **2-11** | **9.0** | **81.6** | **1713** |
| **2-12** | **9.0** | **92.3** | **1857** |
| **2-13** | **8.8** | **94.3** | **1811** |
| **2-14** | **9.5** | **74.7** | **1747** |
| **2-15** | **10.5** | **12.2** | **2418** |
| **2-16** | **9.5** | **36.7** | **2409** |
| **2-17** | **8.2** | **38.5** | **2336** |
| **2-18** | **8.4** | **32.2** | **2422** |
| **2-19** | **8.2** | **38.5** | **2106** |
| **2-20** | **7.0** | **37.5** | **1823** |
| **2-21** | **6.0** | **25.5** | **1648** |
| **2-22** | **5.4** | **47.5** | **1457** |
| **2-23** | **6.3** | **7.0** | **2356** |
| **2-24** | **6.3** | **27.5** | **1565** |
| **2-25** | **8.2** | **72.5** | **1776** |
| **2-26** | **7.0** | **48.5** | **2349** |

No. 2-5 to 2-14 of Table 4 are reference examples. In No. 2-1 to No. 2-4 of Table 4, because the requirement of the present invention was satisfied and the amounts of Ti, Nb and V were properly adjusted in particular, the steel with high strength and excellent in the low temperature toughness could be obtained.

On the other hand, in No. 2-15 to No. 2-24, because at least any one of the requirement of the present invention was not satisfied, the toughness was insufficient.

No. 2-15 to No. 2-19 are the examples in which the C amount was excessive, and the low temperature toughness dropped because the strength increased too high.

In No. 2-20 to No. 2-22, because none of Ti, Nb and V was contained, the grain miniaturizing effect was not exerted, and the low temperature toughness dropped.

Either of No. 2-23 and No. 2-24 is the steel kind equivalent to the standardized steel 9254, and No. 2-24 was subjected to the tempering treatment after quenching. In No. 2-23, the C amount was much and the strength increased excessively, none of Ti, Nb and V was contained, and therefore the low temperature toughness dropped. Also, in No. 2-24, the strength dropped compared with No. 2-23 because the tempering treatment was performed, but the low temperature toughness dropped, because none of Ti, Nb and V was contained.

FIG. 2 is a graph showing the relation between the strength and the low temperature toughness (Charpy absorbed energy at -50°C) with respect to No. 2-1 to 2-24. In FIG. 2, the results of No. 2-1 to 2-14, 2-25 were shown by □, the results of No. 2-15 to No. 2-23, 2-26 were shown by ●, and the result of No. 2-24 was shown by o. According to FIG. 2, it is known that, in all of the steel satisfying the requirement of the present invention (shown by □ in FIG. 2), the Charpy absorbed energy was 50 J/cm² or more and higher toughness was achieved than that in the steel not satisfying any of the requirement of the present invention (shown by ● and o in FIG. 2) when compared with same strength.

## Claims

1. A high-strength spring steel, containing:
C: 0.15-0.33% (means mass%, hereinafter the same);
Si: 1-3.5%;
Mn: 0.20-2.0%; and containing:
at least one element selected from a group consisting of Ti: 0.005-0.10%, Nb: 0.005-0.05% and V: 0.05-0.25%;
Cr: 0.05-1.20%;
P: 0.030% or less;
S: 0.02% or less; and
optionally further containing Ni: 0.05-2% and Cu: 0.05-0.50%; and
optionally further containing B: 0.005% or less and/or Mo: 0.60% or less with the remainder being iron and unavoidable impurities, wherein
a carbon equivalent Ceq₁ expressed by a formula (1) below is 0.55 or less.
Ceq₁=[C]+0.108×[Si]-0.067×[Mn]+0.024×[Cr]-0.05×[Ni]+0.074×[V]...(1) (In the formula (1), each symbol in brackets represents the content (mass%) of the corresponding element.)

2. The high-strength spring steel according to claim 1, containing Ni: 0.15-2%.

3. The high-strength spring steel according to claim 1, containing at least one element selected from a group consisting of Ti: 0.035-0.10%, Nb: 0.005-0.05%, and V: 0.05-0.25%, wherein the grain size number after quenching is 7.5 or above.

4. A method for manufacturing a high-strength spring excellent in corrosion fatigue property, comprising the steps of:
hot-coiling the spring steel according to any one of claims 1-3;
quenching; and
setting thereafter while omitting tempering.

## Patentansprüche

1. Hochfester Federstahl, enthaltend:
C: 0,15-0,33% (bedeutet Massen-%, nachstehend gleich);
Si: 1-3,5%;
Mn: 0,20-2,0%; und enthaltend:
mindestens ein Element, ausgewählt aus einer Gruppe, bestehend aus Ti: 0,005-0,10%, Nb: 0,005-0,05% und V: 0,05-0,25%;
Cr: 0,05-1,20%;
P: 0,030% oder weniger;
S: 0,02% oder weniger; und
gegebenenfalls ferner enthaltend Ni: 0,05-2% und Cu: 0,05-0,50%; und
gegebenenfalls ferner enthaltend B: 0,005% oder weniger und/oder Mo: 0,60% oder weniger, wobei der Rest Eisen und unvermeidbare Verunreinigungen ist,
wobei
ein Kohlenstoffäquivalent Ceq₁, ausgedrückt durch eine nachstehende Formel (1), 0,55 oder weniger beträgt.
Ceq₁=[C]+0,108×[Si]-0,067×[Mn]+0,024×[Cr]-0,05×[Ni]+0,074×[V]...(1) (In der Formel (1) steht jedes Symbol in Klammern für den Gehalt (Massen-%) des entsprechenden Elements.)

2. Hochfester Federstahl nach Anspruch 1, enthaltend Ni: 0,15-2%.

3. Hochfester Federstahl nach Anspruch 1, enthaltend mindestens ein Element, ausgewählt aus einer Gruppe, bestehend aus Ti: 0,035-0,10%, Nb: 0,005-0,05% und V: 0,05-0,25%, wobei die Korngrößenzahl nach dem Abschrecken 7,5 oder höher beträgt.

4. Verfahren zur Herstellung einer hochfesten Feder mit ausgezeichneter Korrosionsermüdungseigenschaft, umfassend die Schritte des:
Warmaufwickelns des Federstahls nach einem der Ansprüche 1 bis 3;
Abschreckens; und
danach Einstellens während das Tempern ausgelassen wird.

## Revendications

1. Acier à ressorts à haute résistance contenant :
C : 0,15 à 0,33 % (% massique moyen, ci-après identique) ;
Si : 1 à 3,5 % ;
Mn : 0,20 à 2,0 % ; et contenant :
au moins un élément sélectionné parmi un groupe constitué de Ti : 0,005 à 0,10 %, Nb : 0,005 à 0,05 % et V : 0,05 à 0,25 % ;
Cr : 0,05 à 1,20 % ;
P : 0,030 % ou moins ;
S : 0,02 % ou moins ; et
contenant en outre en option : Ni : 0,05 à 2 % et Cu : 0,05 à 0,50 % ; et
contenant en outre en option : B : 0,005 % ou moins et/ou Mo : 0,60 % ou moins avec le reste qui est du fer et des impuretés inévitables, dans lequel un carbone équivalent Ceq₁ exprimé par une formule (1) ci-dessous est de 0,55 ou moins.
Ceq¹=[C]+0,108x[Si]-0,067x[Mn]+0,024x[Cr]-0,05x[Ni]+0,074x[V]...(1) (dans la formule (1), chaque symbole entre crochets représente la teneur (% massique) de l'élément correspondant.)

2. Acier à ressorts à haute résistance selon la revendication 1, contenant Ni : 0,15 à 2%.

3. Acier à ressorts à haute résistance selon la revendication 1, contenant au moins un élément sélectionné parmi un groupe constitué de Ti : 0,035 à 0,10 %, Nb : 0,005 à 0,05 % et V : 0,05 à 0,25 %, dans lequel le nombre granulométrique après trempe est de 7,5 ou plus.

4. Procédé de fabrication d'un ressort à haute résistance excellent en termes de propriété de fatigue à la corrosion, comprenant les étapes consistant à :
cintrer à chaud l'acier à ressorts selon l'une quelconque des revendications 1 à 3;
tremper ; et
durcir ci-après tout en omettant le revenu.
